

## 1

3,003,963

## LUBRICATING OIL COMPOSITION

Edward L. Kay, Wappingers Falls, N.Y., assignor to  
 Texaco Inc., a corporation of Delaware  
 No Drawing. Filed Sept. 30, 1958, Ser. No. 764,244  
 2 Claims. (Cl. 252—42.7)

This invention relates to a lubricating composition which is particularly designed for lubrication of modern high speed engines. More particularly, this invention concerns a lubricating oil composition having improved load carrying ability with accompanying resistance to corrosion and coking.

With the improvement and increase in speeds of newly developed heavy high speed machinery, aircraft engines and propulsion engines, it is always desirable to increase the load carrying ability of the lubricating compositions to be used in the lubrication of such engines.

In accordance with the present invention, an improved lubricating composition having increased load carrying ability with excellent corrosion and coking resistance is obtained by the inclusion of from 0.1 to about 5% of a tetra (C<sub>1</sub>—C<sub>6</sub>) alkyl titanate in a lubricating oil. Preferably, a tetra alkyl titanate wherein the alkyl group has from 2 to 4 carbon atoms is used in the preferred amounts of from 0.5 to 1.5 wt. percent.

The tetra alkyl titanates include for example, tetramethyl titanate, tetraethyl titanate, tetrapropyl titanate, tetraisopropyl titanate, tetra-n-butyl titanate and isomers, tetra-n-pentyl titanate and isomers, and tetra-n-hexyl titanate and isomers. Of these tetraethyl, tetrapropyl, tetraisopropyl, tetrabutyl and tetraisobutyl titanates are the preferred additives of the invention.

The lubricating oils of this invention include hydrocarbon lubricating oils and synthetic lubricating oils. The hydrocarbon oils found to be useful for this invention include oils having a viscosity in the range required for lubricating fluids and in particular hydrocarbon mineral oils which include paraffin base, naphthene base, mixed paraffin-naphthene base and residual oils. The hydrocarbon lubricating base generally has been subjected to solvent refining to improve its oxidation and thermal stability and viscosity-temperature properties as well as solvent dewaxing to remove waxy components and to improve the pour of the oil. Broadly speaking, hydrocarbon lubricating oils having an SUS viscosity at 100° F. of between 50 to 2500 are used in the formulation of the improved lubricants of this invention.

The mineral lubricating oils to which the tetra alkyl titanates of this invention are added usually contain other additives designed to impart desirable properties thereto. For example, viscosity index improvers such as the polymethacrylates having a molecular weight ranging from 500 to 25,000 are usually included therein. The VI improver normally used is a polymethacrylate having the following recurring structural unit:



wherein R is an aliphatic radical ranging from butyl to stearyl and n is an integer of more than 1.

## 2

The use of various metal base organic type additives has been found effective and are generally incorporated in the lubricating oils of this invention, particularly those oils used in high speed, spark ignition and diesel engines to reduce ring sticking, minimize lacquer formation and carbon deposits. The metal alkyl phenolates wherein the alkyl group on the benzene nucleus is of comparatively high molecular weight has been found particularly useful where the mineral lubricating oil is of the type generally employed for the crankcase lubrication of aircraft engines which normally operate at higher power levels on high octane airplane fuel. The preferred type of hydroxy aromatic compound is an alkyl phenol prepared by alkylating phenol, cresol, xylenol or other alkyl phenol with an olefin polymer to obtain an alkylated phenol wherein the alkyl constituents on the benzene nucleus contain a total of at least 15 carbon atoms and preferably at least 18 to 30 carbon atoms. A combination of magnesium and zinc salts of alkyl phenols wherein the alkyl groups have from 18 to 30 carbon atoms has been found particularly useful. The magnesium alkyl phenolate is employed within the range of 0.5 to 2.0 wt. percent and the zinc alkyl phenolate is employed in conjunction with the magnesium phenolate in a proportion of 0.25 to 1.5 percent by wt. on the basis of the total lubricating oil composition. Lubricating oil compositions containing the desired combination of magnesium and zinc alkyl phenolates are set forth in U.S. Patent No. 2,674,577 to Frederick C. McCoy, Bill L. Benge, Edwin C. Knowles and Charles C. Towne, issued April 6, 1954.

The hydrocarbon lubricating oils of this invention may also contain other useful additives such as metal sulfonates to afford additional detergent-dispersant properties, metal dialkyl dithiophosphates to afford additional corrosion and oxidation resistance, anti-foam agents such as silicone polymers in the amounts of about 5 to 200 parts per million, etc.

The synthetic lubricating bases are usually of the ester or ether type. High molecular weight, high boiling liquid aliphatic esters generally prepared by reacting 2 moles of a monohydroxy alcohol with an aliphatic dicarboxylic acid, possess excellent viscosity-temperature and lubricating properties and are finding ever increasing utilization in lube oils adapted for high and low temperature lubrication; esters of this type are used in the formulation of jet engine oils. Examples of this class of synthetic lubricating bases are the diesters of acids such as sebacic, adipic, azelaic, alkenyl-succinic, etc.; specific examples of these diesters are di-2-ethylhexyl sebacate, di-2-ethylhexyl azelate, di-2-ethylhexyl adipate, di-n-amyl sebacate, di-2-ethylhexyl n-dodecyl succinate, di-2'-methoxy-2-ethoxyethyl sebacate (the methyl Carbitol diester), di-2'-ethyl-2-n-butoxyethyl sebacate (the 2-ethylbutyl Cellosolve diester), di-2-n-butoxyethyl azelate (the n-butyl Cellosolve diester), and di-2'-n-butoxy-2-ethoxyethyl n-octyl succinate (the n-butyl Carbitol diester).

Polyester lubricants formed by a reaction of an aliphatic dicarboxylic acid of the type previously described, a glycol and an aliphatic monohydroxyl alcohol or an aliphatic monocarboxylic acid in specified mole ratios are also employed as the synthetic lubricating base in the compositions of this invention; polyesters of this type are described in U.S. 2,628,974. Polyesters formed by reaction of a mixture containing specified amounts of di-

propylene glycol, sebacic acid and 2-ethylhexanol and of a mixture containing adipic acid, diethylene glycol and 2-ethylhexanoic acid illustrate this class of synthetic polyester lubricating bases.

Polyalkylene ethers as illustrated by polyglycols are also used as the lubricating base in the compositions of this invention. Polyethylene glycol, polypropylene glycol, polybutylene glycols and mixed polyethylene-polypropylene glycols are examples of this class of synthetic lubricating bases.

The sulfur analogs of the above-described diesters, polyesters and polyalkylene ethers are also used in the formulation of the lubricating compositions of this invention. Dithioesters are exemplified by di-2-ethylhexyl thiosebacate and di-n-octyl thioadipate; polyethylene thioglycol is an example of the sulfur analog of the polyalkylene glycols; sulfur analogs of polyesters are exemplified by the reaction product of adipic acid, thioglycol and 2-ethylhexyl mercaptan.

To demonstrate the excellent improvement in the load-carrying ability of lubricating oils containing the tetra alkyl titanates of this invention, a High Speed Gear Scuff Test was used. This test is intended for the evaluation of the scuff-limited load-carrying ability of those lubricants used in reduction and accessory drives of turbojet and turbo-prop engines. The method of test provides for the running of two spur gears in a Pratt and Whitney Gear and Lubricant Tester (also termed the Ryder Gear Tester). The oil inlet temperature to the gears was  $165^{\circ} \pm 5^{\circ}$  F. The face width of the driven gear was 0.937 inch and the face width of the driving gear was 0.25 inch. The dynamometer speed of the gear tester was 3830 r.p.m. (equivalent to a gear speed of 10,000 r.p.m.) and loading pressure of  $2\frac{1}{2}$  p.s.i. applied during break-in. After running for 10 minutes, the tester was shut down and the driving gear removed and an estimate of the percentage of tooth area scuffed on each tooth of that gear was made. The gear was replaced and the above procedure continuously repeated using a higher loading pressure with increments of 5 p.s.i. at each repetition until 22.5 percent of the total tooth face area on the driving gear had been scuffed, the load corresponding to this point being considered the scuff load. Scuffing is defined as that degree of wear or abrasion which obliterates the axial grinding marks on the gear tooth. The loading pressures used were as follows: 2.5, 5, 10, 15, 20, 25, 30, 35, 40, 45, 50, 55, 60, 65, 70, 75, 80 p.s.i. and up. A tooth load conversion factor of 18.5 sq. in. which was a constant calculated from measured data from the tester, was multiplied by the loading pressure at the scuff load and divided by the width of the driving gear (0.25) to obtain the tooth load in pounds per inch. The results obtained using the above test procedure on various lubricating oil compositions including that of the invention are set forth in the following table:

TABLE I

## High speed gear test

| Oil:                                        | Tooth Load, p.p.i.       |
|---------------------------------------------|--------------------------|
| Base Oil A                                  | 2,640-2,680              |
| Base Oil A+1% (wt.) Tetraisopropyl titanate | 7,400-7,250              |
| Base Oil B                                  | 3,440-3,400              |
| Base Oil B+1% (wt.) Tetraisopropyl titanate | <sup>1</sup> 6,500-7,450 |

<sup>1</sup> No scuff evidenced at this load.

The above table indicates the very great and surprising improvement in the load-carrying ability of the base oil containing tetraisopropyl titanate.

Base oil A consisted of a paraffin base crude residuum which had been propane deasphalting, furfural refined, solvent dewaxed and clay filtered, 16.5% (wt.) of a paraffin base wax distillate which had been furfural refined, light acid treated, solvent dewaxed and clay fil-

tered, and 0.1% (wt.) of a 40% concentrate of a polymerized ester of methacrylic acid having a molecular weight of from 10,000 to 15,000 in a refined mineral oil carrier. The gravity in  $^{\circ}$  API of this base oil composition was 28.2, the SUS viscosity at  $210^{\circ}$  F. was 97.5 seconds, while the viscosity index was 100. Base oil B consisted of base oil A plus 2.9% (wt.) of a mixture of 2 parts of magnesium alkyl phenolate to 1 part zinc alkyl phenolate wherein the alkyl groups contained from 18 to 30 carbon atoms.

The load-carrying ability of the composition of the invention was also demonstrated in the I.A.E. Gear Test which is one of the requirements of British Specification D.E.R.D. 2487, "Lubricating Oil, Aircraft Turbine Engine, Synthetic Type." The I.A.E. Gear Test is also designed to evaluate the scuff-limited, load carrying ability of aircraft gear lubricants.

The results of the I.A.E. Gear Test on lubricating oil compositions of the invention are set forth in the following table:

TABLE II

## I.A.E. gear test

| Oil:                                             | Tooth Load, lbs. |
|--------------------------------------------------|------------------|
| Base Oil A                                       | 80,75            |
| Base Oil A+1% (wt.) tetraisopropyl titanate      | 90,100           |
| Base Oil A plus 3% (wt.) tetraisopropyl titanate | 235,225          |

The above table again indicates the improvement afforded the base oil by the addition of tetraisopropyl titanate. It also shows the further ability of the tetra alkyl titanates of the invention to increase the load-carrying ability of a lubricant composition as greater amounts of titanate are added thereto.

The excellent corrosion resistance of lubricating oil compositions containing the tetra alkyl titanates of the invention was also demonstrated in a number of corrosion tests. The tests were performed using base oils A and C. Base oil C consisted of a paraffin base crude residuum which was propane deasphalting, furfural refined, solvent dewaxed and clay filtered, 3 (wt.) percent of a mixture of 2 parts magnesium alkyl phenolate to 1 part zinc alkyl phenolate wherein the alkyl groups had from 18 to 30 carbon atoms, and 150 parts per million of a 10% dimethyl silicone concentrate in a kerosene carrier as a foam inhibitor.

The S.O.D. Lead Corrosion Test which is described in Military Specification, MIL-L-7808C, Lubricating Oil, Aircraft Turbine Oil, Synthetic Base, dated November 2, 1955, was used to determine the corrosion resistance of lubricating oil compositions of the invention.

Briefly, The S.O.D. Lead Corrosion Test consists of exposing a lead specimen to the action of a test lubricant for one hour at  $325^{\circ}$  F.  $\pm 2^{\circ}$  F. in the presence of a copper catalyst. The test lubricant is mechanically stirred and filtered dry air is introduced into the test lubricant at a controlled rate. Results are presented as change in weight (mgs.) per square inch of lead specimen surface area.

TABLE III

## S.O.D. lead corrosion test

| Oil:                                        | Wt. Loss, mgs. per sq. inch |
|---------------------------------------------|-----------------------------|
| Base Oil A                                  | 0.8                         |
| Base Oil A+1% (wt.) tetraisopropyl titanate | 0.4                         |
| Base Oil C                                  | 0.1                         |
| Base Oil C+1% (wt.) tetraisopropyl titanate | 0.02                        |

The corrosion resistance of the lubricant composition of the invention was also demonstrated in the lead strip corrosion test.

The test consists of exposing a lead specimen to the action of a test lubricant for 48 hours at  $200^{\circ}$  F. under static conditions.

A lead panel consisting of chemically pure lead approximately  $1\frac{1}{8} \times 1\frac{3}{4} \times \frac{1}{32}$  inches is immersed in the test lubricant for 48 hours at a test oil temperature of  $200^{\circ}$  F. A variation of the test is that 2% water is added to the test lubricant and adequately emulsified and the emulsion subjected to above procedure. The test results are expressed as weight change, (mgs.) and are given in the following table:

TABLE IV  
Lead strip corrosion test

| Oil                                         | Wt. Loss, mgs. |               |
|---------------------------------------------|----------------|---------------|
|                                             | Without Water  | With 2% Water |
| Base Oil C                                  | 1              | 70            |
| Base Oil C+1% (wt.) tetraisopropyl titanate | 0              | 35            |

In addition, the corrosion resistance of the lubricant composition of this invention was demonstrated in the MacCoull Corrosion Test. The MacCoull Bearing Corrosion Test is described in S.A.E. Transactions, vol. 50 page 8, August 1952, pages 338-345. The results of the MacCoull Corrosion Test on a lubricating oil composition of the invention is demonstrated in the following table:

TABLE V  
MacCoull bearing corrosion test

| Oil                                         | Cu-Pb<br>Bearing 10 Hr.<br>Wt. Loss, mgs. | Neut.<br>No. |     |
|---------------------------------------------|-------------------------------------------|--------------|-----|
|                                             |                                           | 33.30        | 5.4 |
| Base Oil C                                  | 33.30                                     |              |     |
| Base Oil C+1% (wt.) tetraisopropyl titanate | 0.0                                       | 1.4          |     |

It is obvious from the results set forth in Tables III, IV and V that the tetra alkyl titanates of the invention, as represented by tetraisopropyl titanate, lend much improved corrosion resistance to the lubricating oil composition.

As previously stated, the additives of the invention also unexpectedly lend resistance to coking to lubricating oils. This property is demonstrated in a panel coking test which was initially developed primarily as a test for stability of jet engine oils.

Briefly the test is described as follows: An aluminum panel is polished with emery paper, washed with pe-

roleum ether and weighed. The panel is then heated to  $600^{\circ}$  F. and the test lubricant continuously splashed on to the surface of the panel for a total of 8 hours. Splashing is effected by rotating a spindle at 100 r.p.m. in the test lubricant so that a splashing rate  $2.4 \pm 0.1$  grams per minute is obtained. At the end of 8 hours of splashing, the test panel is removed, cooled and flushed with petroleum ether and reweighed. Any coke deposits on the edges of the test panel shall be removed before final weighing.

10 The following table shows the results of the above described test procedure on lubricating oil compositions of the invention.

TABLE VI  
Panel coking test

| Oil:                                        | Deposits, mgs. |    |
|---------------------------------------------|----------------|----|
|                                             | Base Oil A     | 88 |
| Base Oil A+1% (wt.) tetraisopropyl titanate | 6              |    |
| Base Oil C                                  | 32             |    |
| Base Oil C+1% (wt.) tetraisopropyl titanate | 2              |    |

15 The data presented in the above table are evidence of much improved coking resistance in the lubricating oil composition containing the tetraisopropyl titanate.

20 Obviously, many modifications and variations of the invention as hereinabove described may be made without departing from the spirit and scope thereof, and therefore, only such limitation should be made as are indicated in the appended claims.

25 30 I claim:

1. A mineral lubricating oil containing from about 0.5 to 2% by wt. of a magnesium alkyl phenolate wherein the alkyl group has from 15 to 30 carbon atoms, from about 0.25 to 1.5% by wt. of a zinc alkyl phenolate 35 wherein the alkyl group has from 15 to 30 carbon atoms, and from 0.5 to 1.5% by wt. of a tetra alkyl titanate wherein the alkyl groups have from 2 to 4 carbon atoms.

2. A mineral lubricating oil containing about 3.0 percent by weight of a mixture of 2 parts magnesium alkyl phenolate and 1 part zinc alkyl phenolate wherein the alkyl groups have from 18 to 30 carbon atoms, and from 0.5 to 1.5 percent by weight of tetraisopropyl titanate.

45

References Cited in the file of this patent

UNITED STATES PATENTS

2,160,273 Loane et al. May 30, 1939  
2,674,577 McCoy et al. Apr. 6, 1954